

June 11, 1935.

A. G. LEAKE

2,004,665

METHOD OF TIGHTENING LOOSE RIVETS IN STRUCTURAL MEMBERS

Filed Dec. 30, 1931



Fig. 1



Fig. 2



Fig. 3



Fig. 4

Inventor

Arthur G. Leake

By Worcester & Davis

Attorneys

## UNITED STATES PATENT OFFICE

2,004,665

METHOD OF TIGHTENING LOOSE RIVETS IN  
STRUCTURAL MEMBERS

Arthur G. Leake, Bridgeport, Conn.

Application December 30, 1931, Serial No. 583,816

2 Claims. (Cl. 29—150)

This invention relates to a method of tightening loose rivets in structural members, and has for an object to provide an improved method of so tightening the loosened rivets as to restore 5 their effectiveness without the necessity of removing the rivet or tearing down the structure, and which may be applied while the structure is in position or even under load.

With the foregoing and other objects in view, 10 the invention consists in a certain novel method and means of tightening loose rivets as will be more fully disclosed in connection with the accompanying drawing.

In this drawing:

15 Fig. 1 is a side elevation of a built-up beam or girder showing my invention applied thereto;

Fig. 2 is a vertical section substantially on the line 2—2 of Fig. 1;

Fig. 3 is a top plan view thereof; and

20 Fig. 4 is a detail section on an enlarged scale substantially on the line 4—4 of Fig. 3.

In the drawing the invention is shown as applied to a built-up beam or girder comprising a web plate 10 and angle members 11 secured along 25 the upper and lower edges of the web plate by rivets 12. To the outer surfaces of the longitudinal flanges of the angle members are secured longitudinal strengthening or cover plates 13 by means of rivets 14. It is, however, to be 30 understood that this particular structure is shown merely for the purposes of illustration, and that the invention is equally applicable to tightening loosened rivets in other structures, such as plates, bars, channels, beams, trusses, columns, chords 35 for trusses, webs for plate girders, and all types of built-up structures.

For the purposes of describing the invention we will assume that the rivets 14, or at least a portion of them, have become loosened, and 40 therefore are no longer fully effective as required in the built-up structure. This is illustrated in the drawing, and more particularly in Fig. 4, to an exaggerated extent by showing the shank 15 of the rivet elongated so that the head 16 45 of the rivet does not rest against the surface of the plate 13 when the other head 17 rests against the flange of the angle 11.

The effectiveness of the rivet can be restored and it can be made tight in the structure by welding the outer circumferential portion of the rivet to the surface of the plate 13 or the adjacent structural member as indicated at 18. 5 However, before welding, the surface of the head of the rivet and the surface of the adjacent structural member should be thoroughly cleaned to remove paint, rust, scale and the like. This can be done with an acetylene oxygen torch, 10 cleaning or scraping with a wire brush, or with other suitable cleaning means. Before welding, the head 17 should be held tightly against the adjacent structural member 11, and then the weld metal 18 can be added around the outer 15 periphery of the head 16, it being simultaneously welded to the surface of the head as indicated at 19 and to the surface of the adjacent structural member 13 as indicated at 20. This effectively tightens the rivet and restores its full 20 strength and effectiveness. The weld metal is preferably applied by electric welding from a welding rod, and it will be evident that with this method the rivets can be tightened one at a time without removing any of the rivets, and 25 therefore the rivets can be tightened and restored to full effectiveness while the structural members are in position or under load.

Having thus set forth the nature of my invention, what I claim is:

1. The method of tightening an elongated rivet in structural members which comprises welding in the periphery of one head of the rivet to the member by building up a ring of weld metal 35 around said head between it and the member and welding the ring to the head and the member.

2. The method of tightening an elongated rivet in structural members while under load which comprises holding one head of the rivet tightly 40 against one of the members, and while the rivet is so held welding the periphery of the other head to another member by building up a ring of weld metal around the head between it and the member and welding it to the head and the 45 member.

ARTHUR G. LEAKE.